

## UNITED STATES PATENT OFFICE

HAMILTON D. WAGNON, OF PALOUSE, WASHINGTON

## PROCESS OF MANUFACTURING PAPER PULP

No Drawing.

Application filed February 19, 1929. Serial No. 341,277.

The object of this invention is to effect economies in the process as heretofore followed, said economies to be principally in the composition of the digester liquor, in the time of required cooking, and in the use of the screenings after the cooking process.

I accomplish these objects by means of the process as follows:

The material, preferably straw, is cut into short lengths ready to be deposited in the digester, wherein has previously been deposited the digesting liquid composed of four parts of sal soda to one part of quick lime, to which is added one gallon of hydrocarbon oil for each ton of material to be treated, the resulting liquid being of a specific gravity test known as 2 Baumé scale. Herein lies one of the economies sought to be accomplished, since the digesting liquid heretofore used has been of a specific gravity test of 14 Baumé. To the digesting liquid I add one gallon of hydrocarbon oil, such as kerosene or the like, for each ton of material to be cooked. The object of said oil is to lubricate the fibrous particles of the material, and thus aid in their separation from each other, such aid being observable both in the digester and in the rod mill subsequent to the digester as hereinafter explained.

The use of said oil, and the introduction of the rod mill to be hereinafter explained, so aids in the separation of the fibrous particles as to greatly reduce the required time of cooking in the digester. Heretofore the material has been cooked in the digester for a period of eight hours, but by my process I accomplish the necessary results of the cooking in approximately two hours. Therefore the second economy sought to be accomplished is effected, the reducing of the time for cooking approximately seventy-five percent.

Due to the short period of cooking in the digester, by my process the material is but partially cooked that is in comparison to the present process of much longer cooking, so that while in the present process the fibrous particles are completely separated in the digester, and are thus converted into pulp ready for the paper machine, in my improved

process the fibrous particles are not completely separated. Indeed the cooked material of my process comes from the digester retaining the appearance of the raw material as it entered the digester. However all the cellulose in the material has been dissolved and removed by the cooking.

The cooked material is then deposited within a rod mill, such a device being well known to the art and therefore not described in detail herein. Therein, by the mechanical process of grinding, the fibrous particles are thoroughly separated, and the cooked material reduced to pulp. The above mentioned oil having thoroughly lubricated the fibrous particles greatly facilitates the grinding process within said rod mill.

From the rod mill the pulp is deposited upon a screen, and the screenings, by which will be understood all the material that does not pass through said screen, are again deposited within the rod mill to be further ground. Thus the third economy is accomplished, because all the material is eventually converted into usable pulp, while with the process heretofore used the screenings were more or less waste, being usable only for a very coarse and cheap grade of paper board.

Having disclosed my process so that others may be enabled to follow and use the same, what I claim as new, and desire to secure by Letters Patent is:

The process of manufacturing paper pulp by first cooking the raw material for approximately two hours in a digesting liquid composed of four parts of sal soda to one part of quick lime, diluted to substantially a specific gravity test of two Baumé scale to which is added approximately one gallon of a hydrocarbon oil to each ton of material to be cooked; second subjecting the cooked material to a mechanical separation of the fibrous particles of the material, and thus produce pulp ready for use.

In witness whereof I claim the foregoing as my own I hereunto affix my signature at Portland, county of Multnomah, State of Oregon, this 14th day of Feb., 1929.

HAMILTON D. WAGNON. 100